

Feb. 21, 1967

R. E. BONI ET AL

3,305,354

METHOD OF PRODUCING LOW OXYGEN ORIENTED SILICON-IRON

Filed Dec. 17, 1964



INVENTORS.  
ROBERT E. BONI AND  
JOSEPH E. HECK,  
BY *Youngblut, Melville,  
Stramer & Foster*  
ATTORNEYS.

## 1

3,305,354

**METHOD OF PRODUCING LOW OXYGEN  
ORIENTED SILICON-IRON**

Robert E. Boni, Middletown, and Joseph E. Heck, Monroe, Ohio, assignors to Armco Steel Corporation, Middletown, Ohio, a corporation of Ohio  
Filed Dec. 17, 1964, Ser. No. 419,023  
8 Claims. (Cl. 75—129)

In the manufacture of silicon-iron for magnetic purposes, particularly where the ultimate sheet stock has a preferred orientation, the economic provision of an iron material having initially a low oxygen content or a low content of oxide inclusions has been known to be of great advantage. By way of example, silicon-iron material which is intended for the manufacture of sheet stock having the so-called cube-on-face texture or orientation in which two cube faces or (100) planes are parallel to the sheet surface, should not have at the outset an oxygen content of more than about .0040%. Silicon-iron sheet stocks having the so-called cube-on-edge orientation have improved magnetic properties when made from materials of initially very low oxygen content. Also, although the oxygen may be removed from the solid material during an annealing treatment, this prior technique requires higher temperatures and longer times at temperature.

Hitherto, in the manufacture of silicon-irons of low oxygen values, the best procedures have involved vacuum melting or remelting in the consumable electrode furnace, both of which procedures are relatively expensive. It is an object of this invention to provide a method whereby silicon-irons of other origins can be made in such a way as to have very low oxygen contents at the outset. By the term "other origins" is meant the production of the iron in basic open hearth or electric furnaces, or by those methods in which the molten metal in a suitable container is blown with oxygen.

Silicon-iron is defined for purposes of this invention as being an alloy containing from about 2.5% to about 3.5% of silicon, enough manganese for workability, minor amounts of such elements as carbon, sulfur and phosphorus, the balance being iron with only such impurities as are incident to the mode of manufacture. It has hitherto been suggested that the alloying with the principal alloying elements, silicon and manganese, be accomplished after the metal has been tapped from the furnace in which it was made. While it does not constitute a departure from the spirit of the invention to accomplish part of the alloying in a furnace such as the open hearth and the remainder of the treatment in the ladle from which the molten metal will be teemed into the ingot molds, it is preferred to employ a re-ladling procedure in which part of the treatment is accomplished in a first ladle, after which the molten metal is poured into a second ladle and the remainder of the treatment accomplished therein or during the transfer of the metal from the first ladle to the second. However, it will be understood that whenever mention of additions to first and second ladles or first and second vessels is made in the present specification and claims, the first vessel may be the furnace.

Nevertheless, and particularly in the manufacture of silicon-iron sheet stock having cubic texture, i.e., the special type of cube-on-face orientation designated (100)

## 2

[001] by Miller's Indices, the most consistent results have been attained by (a) vacuum melting or remelting by the use of the consumable electrode furnace, or (b) manufacturing a sheet stock which has another orientation and has been subjected to a final high temperature heat treatment serving to diminish the quantity of oxide inclusions, and then converting such stock to the cubic texture by procedures known in the art.

10 It is an object of this invention to provide a method of making silicon-iron which initially has a very low oxygen content as teemed into the ingot molds, but without resorting to any of the expedients set forth in the preceding paragraph.

15 It is a further object of the invention to provide silicon-iron in cast form which can, by known rolling and annealing steps, be made into either cube-on-edge or cube-on-face oriented sheet stock consistently, at lower cost, and with improved magnetic properties.

20 These and other objects of the invention which will be set forth hereinafter or will be apparent to one skilled in the art upon reading these specifications, are accomplished by that procedure of which exemplary embodiments will now be described. Reference is made to the figure wherein oxygen content in parts per million is plotted against pounds of 65% FeSi added to the first ladle.

25 In the standard procedure in the art it has been the practice to tap the molten metal from the furnace or vessel in which it has been refined into a first ladle and to add to it a relatively small amount of silicon-bearing material, together with manganese-bearing material. For example, the silicon can be added in the form of ferrosilicon, while the manganese can be added in the form of silico-manganese, ferro-manganese, or electrolytic manganese. The term "adding" is used in the broad sense since the alloying elements may be mixed with the molten metal in the furnace, in the tap runner before the metal gets to the first ladle, or placed in the first ladle with the molten metal deposited on top of them. Also, the alloying elements may be fed into the first ladle concurrently with the introduction of the molten metal. The procedure is in any event rapid, and the partially treated metal will not stand longer than two or three minutes after alloying and before transference to the second ladle.

30 40 45 It has been the endeavor in the past to add enough manganese-bearing substance in the first ladle to bring the manganese up to the desired final level which is about .04% to about .12%. At the same time the quantity of silicon-bearing material added to the first ladle has been relatively small and not sufficient to kill the steel.

40 45 In the second ladle, that is to say in any of the ways set forth above, it has been the practice to add the remainder of the silicon-bearing material necessary to raise the silicon value of the alloy to the desired final level.

50 55 Also, it has been the practice to add aluminum to the second ladle for its deoxidizing effect and for ease in pouring. But by the procedure outlined above it has not been possible consistently to produce an alloy containing less than about .010% oxygen.

60 65 By way of contrast the new procedure taught herein contemplates the addition of a very much larger part of the ferrosilicon to the first ladle, together with electrolytic manganese to attain the same final manganese content. Other forms of manganese-bearing material may be used

if desired. In the second ladle the remainder of the silicon-bearing material is added together with somewhat less aluminum than was formerly used.

Surprisingly, the relatively simple change in procedure results in a marked difference in oxygen level in the molten metal. The process of this invention can be depended upon to produce a silicon-iron containing about .0040% or less oxygen.

The contrast between the two procedures is graphically shown in the following chart:

| Old Procedure                                                     |                              | New Procedure                                                                                          |                                                                |
|-------------------------------------------------------------------|------------------------------|--------------------------------------------------------------------------------------------------------|----------------------------------------------------------------|
| First Ladle:                                                      | 100 lbs. 65% ferrosilicon    | First Ladle:                                                                                           | 250-1,250 lbs. 65% ferrosilicon for cube-on-edge stock.        |
| 450-700 lbs. siliconmanganese                                     |                              |                                                                                                        | 750-1,250 lbs. 65% ferrosilicon for cube-on-face stock.        |
| Holding time: None (i.e. no unnecessary delay before re-ladling). |                              |                                                                                                        | 100-575 lbs. manganese (preferably electrolytic).              |
| Second Ladle:                                                     | 15,000 lbs. 65% ferrosilicon | Second Ladle:                                                                                          | Holding time: None or preferably 5 to 15 minutes. <sup>1</sup> |
| 80 lbs. or more aluminum                                          |                              | Balance of the ferrosilicon required to reach desired silicon content (usually less than 15,000 lbs.). |                                                                |
| Holding time: About 20 min.                                       |                              | 60-80 lbs. aluminum.                                                                                   |                                                                |
| Average oxygen about 0.01%                                        |                              | Holding time: About 20 min.                                                                            |                                                                |
|                                                                   |                              | Average oxygen about .0025%.                                                                           |                                                                |

<sup>1</sup> While no holding time after the addition of the alloying ingredients is required beyond the time necessary to transfer the metal to the second ladle, more consistent results are attained with the brief holding times indicated.

10 As will be understood by one skilled in the art, the oxygen content at tap may vary considerably depending upon the refining practice used. In accordance with the new procedure, the amount of ferrosilicon added to the first ladle can be adjusted within the range of 1½ to 8½ lbs. per ton of charge to match the tap oxygen. When it is known that the cast metal will ultimately be made into a cube-on-face product, such as cubic texture, a minimum of about 5 lbs. of 65% ferrosilicon per ton of charge is required. The use of more than 8½ lbs. per ton is unnecessary to obtain the desired low oxygen content.

#### Examples

15 The following table summarizes the procedure and results obtained from 8 exemplary heats of about 150 tons each. The core loss values are not given because the heats were rolled to various final gauges. However, the core losses were found to be lower than those obtained by conventional deoxidizing practices.

| Heat Number | Additions to 1st Ladle, Lbs. |          | Holding Time 1st Ladle, Min. | Additions to 2nd Ladle, Lbs. |      | Holding Time 2nd Ladle, Min. | Ladle Analysis 2nd Ladle, Percent |      |      |      | Percent Oxygen in Ingot (Dip Test) | Percent of Area of Sheet Stock Having Cubic Texture Grains | Straight-Grain Permeability at H=10 Oersteds |
|-------------|------------------------------|----------|------------------------------|------------------------------|------|------------------------------|-----------------------------------|------|------|------|------------------------------------|------------------------------------------------------------|----------------------------------------------|
|             | 65% FeSi                     | Elec. Mu |                              | 65% FeSi                     | Al   |                              | C                                 | Mn   | S    | Si   |                                    |                                                            |                                              |
|             |                              |          |                              |                              |      |                              |                                   |      |      |      |                                    |                                                            |                                              |
| 6534-----   | 250                          | 400      | None                         | 14,900                       | 80   | 20                           | .023                              | .069 | .027 | 3.27 | .0074                              | <sup>1</sup> None                                          | 1,808                                        |
| 2447-----   | 500                          | 575      | None                         | 14,800                       | 80   | 20                           | .026                              | .090 | .028 | 3.15 | .0056                              | <sup>1</sup> None                                          | 1,820                                        |
| 2448-----   | 750                          | 500      | None                         | 14,600                       | 80   | 22                           | .028                              | .124 | .028 | 3.03 | .0030                              | 85-90                                                      | 1,811                                        |
| 6536-----   | 1,000                        | 450      | None                         | 14,400                       | 80   | 20                           | .023                              | .118 | .025 | 3.00 | .0024                              | 100                                                        | 1,803                                        |
| 3248-----   | 1,000                        | 315      | None                         | 15,000                       | None | 20                           | .027                              | .100 | .028 | 3.21 | .0092                              | <sup>1</sup> None                                          | 1,791                                        |
| 5693-----   | 1,100                        | 260      | None                         | 15,300                       | 60   | 25                           | .023                              | .086 | .024 | 3.04 | .0028                              | 100                                                        | 1,797                                        |
| 3093-----   | 1,100                        | 110      | 10                           | 13,000                       | 75   | 20                           | .028                              | .064 | .021 | 2.75 | .0018                              | 100                                                        | 1,831                                        |
| 4536-----   | 1,100                        | 150      | 10                           | 13,700                       | 75   | 20                           | .024                              | .049 | .023 | 2.93 | .0018                              | 100                                                        | 1,828                                        |

<sup>1</sup> Contained very high percentage of cube-on-edge grains.

The figures above are based on heats of about 150 tons each. The total amount of silicon or silicon-bearing material for heats directly compared was the same. Ferrosilicon may be obtained having various percentages of silicon. The above figures are for the 65% ferrosilicon, but these figures can be directly converted for other percentages of ferrosilicon and for other heat sizes. For example, if 90% ferrosilicon were used, only 72% as much would be added to each ladle. Also, if a 300 ton heat were being made, all additions would be doubled.

Based on the weight of the metal treated expressed in short tons (2000 lbs.), the new procedure uses at least 1.67 lbs./ton of 65% ferrosilicon in the first ladle compared with about 0.67 lb./ton in the prior practice, or at least 2½ times as much ferrosilicon per heat in the manufacture of sheet stock capable of being made into cube-on-edge texture silicon-iron. For making a cube-on-face type product, the minimum first ladle addition of ferrosilicon is about 5 lbs./ton of metal, or about 7½ times as much as that formerly used. The maximum ferrosilicon addition necessary for reducing the oxygen content of the metal to less than 6 p.p.m. is about 8.33 lbs./ton of metal, or more than 12 times the amount previously added.

If the aluminum is also expressed in lbs./ton, the addition formerly used was at least .53 lb./ton compared with about .40 to .53 lb./ton in the present practice.

The manganese addition of about 100 to 575 pounds of electrolytic manganese for a heat of 150 tons may be expressed as about 0.67 to 3.84 lbs./ton of metal.

The ferrosilicon used in the practice of this invention

45 It will be apparent that the new practice of increasing the deoxidation by silicon in the first ladle lowers considerably the final oxygen content of the ingot or hot band. Yet, as noted by the results for Heat 3248, it has been found that aluminum must still be added to the second ladle. This synergistic effect of the combination of silicon and aluminum has not been heretofore recognized.

55 The reasons for the unexpected and surprising results obtained by the practice of this invention are obscure. Without wishing to be bound by theory, it nevertheless appears that aluminum as a getter for oxygen at the low oxygen levels involved here is not effective unless the molten metal has first been treated with a very substantial quantity of silicon, and in particular with enough silicon-bearing material to leave a substantial residual quantity of silicon in alloyed condition in the ferrous metal. A laboratory study indicated that aluminum serves to increase the rate of deoxidation of silicon-iron. By the same token, the process of this invention operates to give a lower final oxygen content with the use of less aluminum.

60 65 The holding times as set forth for the new procedure have been found beneficial in permitting oxide inclusions such as silicates and aluminates and their combinations with other oxides to float upwardly to the top of the metal bath. The prior practice of re-ladling as soon as the first ladle is full may not allow enough time for the effective deoxidation and removal of the resulting inclusions. The kinetics of the deoxidation reactions and the removal of the inclusions by flotation have not been studied. If these impurities are not removed in the furnace or first

ladle, they will be carried into the teeming ladle and from there into the casting. If sufficient additional ferrosilicon is added to the melting furnace to lower the oxygen content of the melt to a level requiring only a single ladle, this ladle should be held for about 20 minutes before the metal is teemed into molds or poured into a continuous casting machine.

The embodiments of the invention in which an exclusive property or privilege is claimed are defined as follows:

1. A method of producing low oxygen silicon-iron intended for the manufacture of oriented silicon-iron sheet stock, comprising the steps of adding to molten ferrous metal in a first vessel a quantity of silicon-bearing material sufficient to combine with oxygen in the ferrous metal and to leave a substantial residual quantity of silicon in alloyed condition in the ferrous metal, adding a quantity of manganese-bearing material to said first vessel sufficient to bring the manganese content of said ferrous metal up to a desired final level, transferring said ferrous metal to a second vessel, adding a quantity of said silicon-bearing material sufficient to bring the silicon content of said ferrous metal to a desired final alloy level, adding aluminum to said ferrous metal, and holding said ferrous metal in said second vessel for a holding period sufficient to allow inclusions to float out of said ferrous metal.

2. The process claimed in claim 1 wherein said ferrous metal is held in both vessels and the holding period for said first vessel is about 5-15 minutes and the holding period for said second vessel is about 20 minutes.

3. The process claimed in claim 1 wherein the ferrous

metal charge is subsequently made into a sheet product having a cube-on-edge orientation and wherein the silicon-bearing material added to the first vessel is ferrosilicon added in a quantity equivalent to at least 1½ pounds of 65% ferrosilicon per ton of said metal charge.

4. The process claimed in claim 1 wherein the ferrous metal charge is subsequently made into a sheet product having a cube-on-face crystallographic orientation and wherein the equivalent of at least 5 pounds of 65% ferrosilicon is added to the first vessel per ton of said metal charge.

5. The process claimed in claim 3 wherein the said manganese addition to said first vessel is equivalent to about ⅔ pound to 4 pounds of manganese per ton of metal charge.

6. The process claimed in claim 3 wherein said aluminum addition to said ferrous metal in said second vessel is equivalent to about ⅔ pound to about ½ pound per ton of metal charge.

7. The process claimed in claim 4 wherein the said manganese addition to said first vessel is equivalent to about ⅔ pound to 4 pounds of manganese per ton of metal charge.

8. The process claimed in claim 4 wherein said aluminum addition to said ferrous metal in said second vessel is equivalent to about ⅔ to about ½ pound per ton of metal charge.

No references cited.

30 BENJAMIN HENKIN, Primary Examiner.